

## 1

3,732,104

**SILVER HALIDE EMULSIONS CONTAINING AZAINDENE AND AMIDE STABILIZING AGENTS**

Hubert Vandenabeele, Wilrijk, Joseph Louis De Munck, Heide-Kalmthout, Robrecht Julius Thiers, Brasschaat, Robert Joseph Pollet, Vremde, Raymond Leopold Florens, Edegem, and Jozef Frans Willems, Wilrijk, Belgium, assignors to Gevaert-Agfa, N.V., Mortsel, Belgium

No Drawing. Filed Oct. 27, 1970, Ser. No. 84,489  
Claims priority, application Great Britain, Nov. 3, 1969,  
53,825/69

Int. Cl. G03c 1/34

U.S. Cl. 96—109

12 Claims

**ABSTRACT OF THE DISCLOSURE**

Photographic materials comprising a light-sensitive silver halide emulsion element containing an azaindene emulsion stabilizing agent in contact with as an additional stabilizing agent an amide having the formula:



wherein

each of  $R_1$  and  $R_2$  stands for hydrogen, lower alkyl, lower alkyl carrying a hydroxyl group, lower alkyl carrying the group  $R_3CONH-$ , or a phenyl group,  $R_1$  together with  $R_2$  stands for the atoms necessary to close a pyrrolidine, piperidine or morpholine nucleus,  $R_3$  stands for lower alkyl or the group



wherein each of  $R'_1$  and  $R'_2$  have the same significance as  $R_1$  and  $R_2$ ,  $R'_1$  and  $R'_2$  both being different from hydrogen, or  $R_3$  may represent hydrogen when  $R_1$  or  $R_2$  is substituted alkyl, or  $R_3$  together with  $R_2$  stands for alkylene.

A synergistic effect is obtained with regard to fog inhibition particularly upon storage of the element.

This invention relates to improved photographic materials comprising light-sensitive silver halide emulsions, more particularly to photographic materials having less tendency to fog formation and showing no appreciable desensitization upon storage.

It is well known that light-sensitive silver halide materials comprising gelatin silver halide emulsion layers are subject to fogging. Fogging in general and chemical fogging in particular may be defined as the formation of a uniform deposit of silver on processing which is dependent on a whole series of circumstances and factors namely on the nature of the emulsions, on their age, on the conditions under which they have been stored, on the processing conditions, etc. For particular processing conditions the fog tends to be greater as the time of storage and the temperature and relative humidity of the atmosphere, in which the emulsions are stored, are increased.

Addenda to the photographic material known as stabilizers or antifogants protect the light-sensitive silver

## 2

halide emulsions against formation and growth of fog particularly in high-sensitive emulsions and in emulsions which are stored under adverse conditions of temperature and humidity as is for instance the case in tropical countries. Among these addenda the azaindene stabilizing agents are widely used because of their unique properties in stabilizing the emulsions against the development of this general fog without giving rise to an appreciable desensitization.

It has now been found that the stability of light-sensitive silver halide emulsions comprising azaindene stabilizing agents against growth of fog can still be improved by the use of amide compounds corresponding to the formula:



or polymers comprising recurring units of the formula:



wherein

each of  $R_1$  and  $R_2$  stands for hydrogen, alkyl preferably comprising at most 5 C-atoms including substituted alkyl such as hydroxylalkyl and the group  $R_3CONH-$ alkyl, or aryl including substituted aryl, or  $R_1$  together with  $R_2$  represent the atoms necessary to close a pyrrolidine, piperidine or morpholine nucleus,  $R_3$  stands for alkyl preferably comprising at most 5 C-atoms, for the group



wherein each of  $R'_1$  and  $R'_2$  have the same significance as  $R_1$  and  $R_2$ ,  $R'_1$  and  $R'_2$  both being different from hydrogen however, or  $R_3$  may represent hydrogen when  $R_1$  or  $R_2$  stands for substituted alkyl in particular  $R_3CONH$ -alkyl,

or  $R_3$  together with  $R_2$  stand for alkylene, preferably alkylene comprising at least 3 methylene groups such as pentamethylene,  $R_1$  then being preferably hydrogen, and

$R_4$  stands for hydrogen or lower alkyl such as methyl, as additional stabilizing agents, the sensitivity not being influenced to a noteworthy extent.

Thus, in accordance with the present invention photographic emulsions are provided which are stabilized with azaindene and additionally stabilized with amide compounds corresponding to the above general formulae.

Exemplary compounds corresponding to the above general formulae that are suitable for use with azaindene stabilizing agents in light-sensitive silver halide emulsions are:

 (1) acetamide  $H_3CCONH_2$ 


65

- (3) dihydroxyethyl acetamide  $\text{H}_3\text{CCON}(\text{CH}_2\text{CH}_2\text{OH})_2$
- (4) tetramethylurea  $\text{H}_3\text{C}-\text{N}(\text{CONH}_2)-\text{CH}_3$
- (5) propionamide  $\text{CH}_3\text{CH}_2\text{CONH}_2$
- (6) butyramide  $\text{CH}_3\text{CH}_2\text{CH}_2\text{CONH}_2$
- (7)  $\epsilon$ -caprolactam  $\text{H}_2\text{C}-\text{CH}_2-\text{CO}-\text{CH}_2-\text{CH}_2-\text{NH}-\text{CH}_2-\text{CH}_2-\text{CH}_2$
- (8) poly(*N*-acrylmorpholine) having recurring units of the formula:



and having an intrinsic viscosity of 0.134 dl./g.<sup>-1</sup> measured at 25° C. in tetrahydrofuran, prepared by refluxing a 10% by weight solution in methanol of the monomer in the presence of 5% by weight relative to the monomer of azobisisobutyronitrile as initiator.

- (9) acetanilide  $\text{H}_3\text{CCONH}-\text{C}_6\text{H}_4-\text{CH}_3$
- (10)  $\text{OHCNHCH}_2\text{CH}_2\text{NHCHO}$

The amide compounds of use according to the present invention are preferably incorporated into the silver halide emulsion layer comprising azaindene stabilizer of the light-sensitive material. The way in which the azaindene and amide compounds of use according to the invention are added to emulsions is not critical and the addition may occur during no matter what step of emulsion preparation.

The preparation of silver halide emulsions involves three separate operations: (1) the emulsification and digestion or ripening of the silver halide, (2) the freeing of the emulsion from aqueous soluble salts usually by washing, and (3) the second digestion or after ripening (chemical ripening) to obtain increased sensitivity.

The azaindene and amide compounds of use according to the present invention can be added before or after the emulsion has been optically sensitized, preferably just before coating of the emulsion on a suitable support such as for example paper, glass or film such as cellulose triacetate and polyethylene terephthalate.

Instead of incorporating the amide compounds of the invention into the emulsion layer comprising azaindene stabilizer they can also be incorporated into another layer of the photographic material, e.g. a gelatin anti-stress layer or intermediate layer, which is in water-permeable relationship with the said emulsion layer or into one of the processing baths for said photographic material.

The amide stabilizers of use according to the present invention may be used in conjunction with azaindene stabilizers in any type of light-sensitive material e.g. spectrally sensitized or non-sensitized silver halide material, silver halide material of use in diffusion transfer processes for the production of silver images, and X-ray material. They may be used in high speed negative materials as well as into rather low speed positive materials. Various silver salts may be used as light-sensitive salt e.g. silver bromide, silver iodide, silver chloride, or mixed silver halides e.g. silver chlorobromide or silver bromoiodide.

The silver halides are dispersed in the common hydrophilic colloids such as gelatin, casein, zein, polyvinyl alcohol, carboxymethylcellulose, alginic acid, etc., gelatin being, however, favoured.

The amount of amide compound employed in the light-sensitive silver halide material depends on the particular type of emulsion and the desired effect and can vary within very wide limits. The optimum amount of amide compound to be added is best determined for each particular type of emulsion by trial. Generally, the most suitable concentration is between 0.5 g. and 20 g. of amide compound per mole of silver halide.

The azaindene stabilizing agents used in the silver halide emulsions in concentrations as known in the art which are of the order of from 0.02 gram to 10.0 grams, preferably from 0.1 and 5 g. per mole of silver halide.

Azaindene stabilizing agents for use in light-sensitive silver halide material are widely known in the art. Examples of azaindene stabilizing agents can be found in literature amongst others in U.S. Pat. 2,944,902 and the patent literature referred to therein for that purpose. They include amongst others the hydroxy tetraazaindene corresponding to the formula:



wherein:

each of  $\text{R}_4$  and  $\text{R}_5$  stands for hydrogen, alkyl, aralkyl and aryl, and  
 $\text{R}_6$  stands for hydrogen, alkyl, carboxy or alkoxy carbonyl.

By way of example, 5-methyl-7-hydroxy-s-triazolo[1,5-a]pyrimidine, 6-carboxy-7-hydroxy-s-triazolo[1,5-a]pyrimidine, 6 - carbethoxy - 7 - hydroxy-s-triazolo[1,5-a]pyrimidine and 2- $\beta$ -hydroxyethyl-5-methyl-7-hydroxy-s-triazolo[1,5-a]pyrimidine can be mentioned as suitable hydroxy tetraazaindenes.

The light-sensitive emulsions may be chemically as well as optically sensitized. They may be chemically sensitized by any of the accepted procedures. The emulsions may be digested with naturally active gelatin or sulphur compounds may be added such as allyl thiocyanate, allyl thiourea, sodium thiosulphate, etc. The emulsions may also be sensitized by means of reductors for instance tin compounds as described in our British patent specification 789,823 and by means of small amounts of noble metal compounds such as of gold, platinum, palladium, iridium, ruthenium and rhodium. Representative compounds are ammonium chloro palladate, potassium chloroplatinate, potassium chloroaurate and potassium aurithiocyanate. These sensitizers can be added during no matter what step of emulsion preparation e.g. before, during or after the chemical ripening.

Other addenda such as hardening agents e.g. formaldehyde, dialdehydes, halogen substituted aldehyde acids such as mucochloric and mucochromic acid, etc., wetting agents, plasticizers, colour couplers, developing agents and optical sensitizers can be incorporated into the emulsion in the usual way.

The azaindene and amide compounds of use according to the present invention are particularly suitable for use in conjunction with compounds which sensitize the emulsion by development acceleration for example alkylene oxide polymers. These alkylene oxide polymers may be of various type. Various derivatives of alkylene oxides may be used to sensitize the silver halide emulsions, e.g. alkylene oxide condensation products as described among others in United States patent specifications 2,531,832 and 2,533,990, in United Kingdom patent specifications

920,637, 940,051, 945,340 and 991,608 and in Belgian patent specification 648,710. Other compounds that sensitize the emulsion by development acceleration and that are suitable for use in combination with the azaindene and amide compounds of use according to the invention are the onium derivatives of amino-N-oxides as described in United Kingdom patent specification 1,121,696.

The emulsions may further comprise other known antifoggants or stabilizers for instance heterocyclic nitrogen containing thioxo compounds such as benzothia-

Development occurred for 6 min. at 20° C. in a developing bath having the following composition:

|                                   |    |     |
|-----------------------------------|----|-----|
| Water                             | ml | 800 |
| p-Monomethylamino phenol sulphate | g  | 4   |
| Sodium sulphite (anhydrous)       | g  | 65  |
| Hydroquinone                      | g  | 10  |
| Sodium carbonate (anhydrous)      | g  | 45  |
| Potassium bromide                 | g  | 5   |
| Water to make 1000 ml.            |    |     |

TABLE

| Compound(s) added per kg.<br>emulsion | Fresh material |          |                | Stored material |          |                |
|---------------------------------------|----------------|----------|----------------|-----------------|----------|----------------|
|                                       | Fog            | $\gamma$ | Relative speed | Fog             | $\gamma$ | Relative speed |
| 0.600 g. of azaindene 1 (a)           | 0.04           | 2.30     | 100            | 0.15            | 1.93     | 105            |
| 8 g. of compound 1 (b)                | 0.07           | 2.59     | 145            | 2.85            |          |                |
| (a) plus (b)                          | 0.03           | 2.46     | 102            | 0.11            | 2.12     | 107            |
| 8 g. of compound 6 (c)                | 0.06           | 2.58     | 145            | 2.88            |          |                |
| (a) plus (d)                          | 0.03           | 2.63     | 102            | 0.11            | 2.30     | 110            |
| 8 g. of compound 3(d)                 | 0.09           | 2.34     | 200            | 3.15            |          |                |
| (a) plus (b)                          | 0.02           | 2.62     | 105            | 0.13            | 2.25     | 126            |
| 8 g. of compound 5(e)                 | 0.08           | 2.43     | 123            | 2.51            |          |                |
| (a) plus (e)                          | 0.03           | 2.60     | 100            | 0.12            | 2.30     | 110            |
| 8 g. of compound 8(f)                 | 0.74           | 2.00     | 81             | 2.15            |          |                |
| (a) plus (f)                          | 0.08           | 2.90     | 123            | 0.11            | 2.49     | 118            |

<sup>1</sup> The azaindene stabilizer used in the above materials is 5-methyl-7-hydroxy-s-triazolo [1,5-a] pyrimidine.

zoline-2-thione and 1-phenyl -  $\Delta_2$  - tetrazoline-5-thione, mercury compounds such as those described in Belgian patent specifications 525,121 and 677,337 and in Belgian patent specifications 707,386 and 709,195 and salts such as cadmium chloride, cadmium nitrate, cobalt nitrate, manganese chloride, zinc chloride and zinc nitrate, sulphuric acids such as benzene sulphuric acid and toluene sulphuric acid, thiosulphonic acids such as benzene thiosulphonic acid, toluene thiosulphonic acid, p-chloro-benzene thiosulphonic acid sodium salt, propyl thiosulphonic acid potassium salt, butyl thiosulphonic acid potassium salt, etc. These thiosulphonic acid compounds are particularly suitable for use in emulsions ripened

30 From the above results appears that when using in azaindene stabilized emulsions the amide compounds according to the invention fog formation is still reduced, especially upon storage, though these compounds, when used alone, give high fog values upon storage.

## EXAMPLE 2

35 Example 1 is repeated with the difference, however, that development now took place for 20 sec. at 40° C. in the tanning 1 - phenyl - 3-pyrazolidinone/hydroquinone developer "G 137" marketed by Gevaert-Agfa N.V. Belgium.

The sensitometric results attained are listed in the table 40 below.

| Compound(s) added per kg.<br>emulsion              | Fresh material |           |                | Stored material |           |                |
|----------------------------------------------------|----------------|-----------|----------------|-----------------|-----------|----------------|
|                                                    | Fog            | Gradation | Relative speed | Fog             | Gradation | Relative speed |
| 0.600 g. of the azaindene compound of example 1(a) | 0.05           | 1.87      | 100            | 0.12            | 1.29      | 63             |
| (a) plus 8 g. of compound 1                        | 0.03           | 2.01      | 102            | 0.09            | 1.33      | 71             |
| (a) plus 8 g. of compound 3                        | 0.03           | 1.95      | 102            | 0.08            | 1.59      | 93             |
| (a) plus 8 g. of compound 5                        | 0.02           | 2.08      | 105            | 0.09            | 1.41      | 72             |
| (a) plus 8 g. of compound 6                        | 0.03           | 2.19      | 107            | 0.09            | 1.47      | 76             |
| (a) plus 8 g. of compound 8                        | 0.06           | 1.77      | 73             | 0.07            | 1.59      | 60             |

55 with noble metal compounds or reducing agents and are, unlike the sulphuric acids, fully compatible with hardening by means of mucochloric and mucobromic acid.

The following examples illustrate the present invention.

## EXAMPLE 1

An orthochromatic ammoniacal silver bromoiodide emulsion (2.75% of iodide), for photography of the green fluorescent screen, which comprises per kg. an amount of silver halide equivalent to 180 g. of silver nitrate and 72 g. of gelatin, was divided into several portions. To each of these portions the compounds listed in the table below were added in the amount given, prior to coating on a conventional film support.

The values of speed, gradation and fog of the materials formed were determined shortly after preparation and after having been stored for 36 hours at 57° C. and 34% relative humidity.

These values are listed in the table below. The values of the speed are relative values with respect to the speed of the material comprising only 5-methyl-7-hydroxy-s-triazolo[1,5-a]pyrimidine to which the value 100 is given (fresh material).

55 From these results too it appears that the amide compounds of the invention reduce fog formation in azaindene-stabilized emulsions.

## EXAMPLE 3

A gelatino silver bromoiodide emulsion (2 mole percent of iodide) comprising per kg. an amount of silver halide equivalent to 180 g. of silver nitrate and 72 g. of gelatin was divided into several portions. To each of these portions the compounds listed in the table below were added in the amount given, prior to coating on a conventional film support.

65 The values of speed, gradation and fog of the materials formed were determined shortly after preparation and after having been stored for 36 hours at 57° C. and 34% of relative humidity by exposure to X-rays with an X-ray radiation source of 80 kv. and development for 4 min. at 20° C. in a common X-ray developer having the composition given in Example 1.

70 The values attained are listed in the table below. The values of the speed are relative values with respect to the speed of the material comprising only 5-methyl-7-hydroxy-s-triazolo[1,5-a]pyrimidine to which the value 100 is given (fresh material).

| Compound(s) added per kg.<br>emulsion                        | Fresh material |                |                   | Stored material |                |                   |
|--------------------------------------------------------------|----------------|----------------|-------------------|-----------------|----------------|-------------------|
|                                                              | Fog            | Grada-<br>tion | Relative<br>speed | Fog             | Grada-<br>tion | Relative<br>speed |
| 0.600 g. of the azaindene com-<br>ound of Example 1 (a)----- | 0.11           | 2.88           | 100               | 0.24            | 2.16           | 128               |
| 2 g. of compound 1 (b)-----                                  | 0.10           | 2.59           | 128               | >2.00           | -----          | -----             |
| (a) plus (b)-----                                            | 0.07           | 2.96           | 104               | 0.12            | 2.32           | 132               |
| 10 g. of compound 2 (c)-----                                 | 0.16           | 2.52           | 114               | >2.00           | -----          | -----             |
| (a) plus (c)-----                                            | 0.07           | 3.00           | 110               | 0.16            | 2.29           | 132               |
| 10 g. of compound 4 (d)-----                                 | 0.15           | 2.42           | 128               | >2.00           | -----          | -----             |
| (a) plus (d)-----                                            | 0.09           | 2.78           | 112               | 0.20            | 2.10           | 126               |
| 10 g. of compound 5 (e)-----                                 | 0.09           | 2.57           | 128               | >2.00           | -----          | -----             |
| (a) plus (e)-----                                            | 0.03           | 3.10           | 117               | 0.13            | 2.41           | 144               |

## EXAMPLE 4

Example 3 is repeated with the difference, however, that development took place for 20 sec. at 40° C. in the tanning 1 - phenyl - 3 - pyrazolidinone/hydroquinone developer "G 137" marketed by Gevaert-Agfa N.V., Mortsel, Belgium.

The results attained are listed below.

with the said emulsion layer as an additional stabilizing agent an amide compound corresponding to the formula:



20

| Compound(s) added per kg.<br>emulsion                   | Fresh material |                |                   | Stored material |                |                   |
|---------------------------------------------------------|----------------|----------------|-------------------|-----------------|----------------|-------------------|
|                                                         | Fog            | Grada-<br>tion | Relative<br>speed | Fog             | Grada-<br>tion | Relative<br>speed |
| 0.600 g. of azaindene compound<br>of Example 1 (a)----- | 0.28           | 1.90           | 100               | 0.32            | 1.50           | 112               |
| 2 g. of compound 1 (b)-----                             | 0.28           | 1.55           | 112               | >3.00           | -----          | -----             |
| (a) plus (b)-----                                       | 0.13           | 1.87           | 100               | 0.21            | 1.46           | 100               |
| 10 g. of compound 2 (c)-----                            | 0.36           | 1.50           | 78                | >3.00           | -----          | 98                |
| (a) plus (c)-----                                       | 0.13           | 1.90           | 98                | 0.26            | 1.44           | 98                |
| 10 g. of compound 4 (d)-----                            | 0.29           | 1.50           | 100               | >3.00           | -----          | -----             |
| (a) plus (d)-----                                       | 0.18           | 1.85           | 107               | 0.26            | 1.34           | 88                |
| 10 g. of compound 5 (e)-----                            | 0.37           | 1.48           | 78                | >3.00           | -----          | -----             |
| (a) plus (e)-----                                       | 0.07           | 2.00           | 107               | 0.23            | 1.42           | 100               |

## EXAMPLE 5

Examples 3 and 4 are repeated and the results attained are listed in the following tables.

wherein:

each of R<sub>1</sub> and R<sub>2</sub> stands for hydrogen, lower alkyl, lower alkyl carrying a hydroxyl group, lower alkyl carrying

## 1. After development as described in Example 3

| Compound(s) added per kg.<br>emulsion                       | Fresh material |                |                   | Stored material |                |                   |
|-------------------------------------------------------------|----------------|----------------|-------------------|-----------------|----------------|-------------------|
|                                                             | Fog            | Grada-<br>tion | Relative<br>speed | Fog             | Grada-<br>tion | Relative<br>speed |
| 0.00 g. of the azaindene com-<br>ound of Example 1 (a)----- | 0.20           | 3.52           | 100               | 0.30            | 2.74           | 142               |
| 10 g. of compound 1 (b)-----                                | 0.2            | 3.30           | 76                | 1.70            | -----          | -----             |
| (a) plus (b)-----                                           | 0.09           | 3.35           | 96                | 0.18            | 2.62           | 142               |
| 10 g. of compound 9 (c)-----                                | 0.1            | 3.35           | 81                | 1.80            | -----          | -----             |
| (a) plus (c)-----                                           | 0.13           | 3.30           | 102               | 0.20            | 2.54           | 152               |

## 2. After development as described in Example 4

| Compound(s) added per kg.<br>emulsion                        | Fresh material |                |                   | Stored material |                |                   |
|--------------------------------------------------------------|----------------|----------------|-------------------|-----------------|----------------|-------------------|
|                                                              | Fog            | Grada-<br>tion | Relative<br>speed | Fog             | Grada-<br>tion | Relative<br>speed |
| 0.600 g. of the azaindene com-<br>ound of Example 1 (a)----- | 0.65           | 3.30           | 100               | 1.48            | -----          | -----             |
| 10 g. of compound 1 (b)-----                                 | 1.25           | 3.30           | 95                | 2.30            | -----          | -----             |
| (a) plus (b)-----                                            | 0.40           | 3.30           | 95                | 0.54            | 2.10           | 110               |
| 10 g. of compound 9 (c)-----                                 | 1.40           | 3.24           | 102               | 2.20            | -----          | -----             |
| (a) plus (c)-----                                            | 0.40           | 3.24           | 102               | 0.40            | 2.16           | 132               |

We claim:

1. Photographic material comprising a light-sensitive, developing-out, silver halide emulsion layer containing an azaindene emulsion stabilizing agent having the formula:



wherein:  
each of R<sub>4</sub> and R<sub>5</sub> stands for hydrogen, alkyl, aralkyl and aryl, and R<sub>6</sub> stands for hydrogen, alkyl, carboxy or alkoxy carbonyl,

said material comprises in the said emulsion layer or in another colloid layer in water-permeable relationship

R<sub>1</sub> together with R<sub>2</sub> stands for the atoms necessary to close a pyrrolidone, piperidine or morpholine nucleus, R<sub>3</sub> stands for lower alkyl or the group



65 wherein each of R'<sub>1</sub> and R'<sub>2</sub> have the same significance as R<sub>1</sub> and R<sub>2</sub>, R'<sub>1</sub> and R'<sub>2</sub> both being different from hydrogen, or R<sub>3</sub> may represent hydrogen when R<sub>1</sub> or R<sub>2</sub> is substituted alkyl, or

R<sub>3</sub> together with R<sub>2</sub> stands for alkylene.

2. Photographic material according to claim 1, where-  
in said amide compound corresponds to the formula:



wherein:

$R_1$  stands for hydrogen, and  
 $R_3$  together with  $R_2$  stands for alkylene.

3. Photographic material according to claim 1, wherein said amide compound corresponds to the formula:



wherein:

$R_1$  stands for hydrogen or lower alkyl,  
 $R_2$  stands for lower alkyl carrying the group  $R_3\text{CONH}-$ , and  
 $R_3$  stands for hydrogen or lower alkyl.

4. Photographic material according to claim 1, wherein said amide compound is present in the azaindene stabilized emulsion layer.

5. Photographic material according to claim 1, wherein said azaindene is 5-methyl-7-hydroxy-s-triazolo pyrimidine.

6. Photographic material according to claim 1, wherein the said emulsion layer comprises a development accelerator of the polyoxyalkylene type.

7. Photographic material according to claim 1 wherein said amide compound corresponds to the formula:



wherein:

each of  $R_1$  and  $R_2$  stands for hydrogen, lower alkyl, hydroxy-substituted lower alkyl, or phenyl, and  
 $R_3$  stands for lower alkyl, or



each of  $R'_1$  and  $R'_2$  being lower alkyl, hydroxy-substituted lower alkyl or phenyl.

8. Process for inhibiting fog-formation in photographic silver halide materials comprising a support carrying water-permeable colloid layers including a silver halide emulsion layer, which comprises an azaindene emulsion stabilizing agent having the formula:



wherein:

each of  $R_4$  and  $R_5$  stands for hydrogen, alkyl, aralkyl and aryl, and  $R_6$  stands for hydrogen, alkyl, carboxy or alkoxy carbonyl,

which process comprises processing the said material after image-wise exposure in the presence of an amide compound corresponding to the formula:



wherein:

each of  $R_1$  and  $R_2$  stands for hydrogen, lower alkyl group, lower alkyl carrying a hydroxyl group, lower alkyl carrying the group  $R_3\text{CONH}-$ , or a phenyl group,

$R_1$  together with  $R_2$  stands for the atoms necessary to close a pyrrolidone, piperidine or morpholine nucleus,  $R_3$  stands for lower alkyl or the group



wherein each of  $R'_1$  and  $R'_2$  have the same significance as  $R_1$  and  $R_2$ ,  $R'_1$  and  $R'_2$  both being different from hydrogen, or  $R_3$  may represent hydrogen when  $R_1$  or  $R_2$  is substituted alkyl, or  
 $R_3$  together with  $R_2$  stands for alkylene.

9. Process according to claim 8, wherein said amide compound corresponds to the formula:



wherein:

10  $R_1$  stands for hydrogen, and  
 $R_3$  together with  $R_2$  stands for alkylene.

10. Process according to claim 8, wherein the said azaindene is 5-methyl-7-hydroxy-s-triazolo pyrimidine.

11. Process according to claim 8, wherein said amide compound corresponds to the formula:



30 wherein:

$R_1$  stands for hydrogen or alkyl,  
 $R_2$  stands for the group  $R_3\text{CONH}-$ , and  
 $R_3$  stands for hydrogen or alkyl.

35 12. Process according to claim 8 wherein said amide compound corresponds to the formula:



wherein:

each of  $R_1$  and  $R_2$  stands for hydrogen, lower alkyl, hydroxy-substituted lower alkyl or phenyl, and

45  $R_3$  stands for lower alkyl, or



50 each of  $R'_1$  and  $R'_2$  being lower alkyl, hydroxy-substituted lower alkyl or phenyl.

#### References Cited

##### UNITED STATES PATENTS

3,333,959 8/1967 Hayakawa et al. ----- 96—109  
 3,486,901 12/1969 Karlson ----- 96—109

##### FOREIGN PATENTS

350,996 6/1931 Great Britain ----- 96—109

NORMAN G. TORCHIN, Primary Examiner

65 W. H. LOUIE, JR., Assistant Examiner

U.S. CL. X.R.

96—66.5

UNITED STATES PATENT OFFICE  
CERTIFICATE OF CORRECTION

Patent No. 3,732,104 Dated May 8, 1973

Inventor(s) HUBERT VANDENABEELE ET AL Page 1 of 2

It is certified that error appears in the above-identified patent and that said Letters Patent are hereby corrected as shown below:

Column 2, lines 15 - 18, the formula should appear as follows:



Column 3, line 16, "poly(N-acrylmorpholine)" should read -- poly(N-acryloylmorpholine) --; Column 3, line 27, "0.134 dl./g.  $\text{-}^1$ " should read -- 0.134 dl g $^{-1}$  --. Column 5, line 30, "525,121" should read -- 524,121 --. Column 6, lines 12 - 25, in the Table, column 1, compound 5, "(a) plus (d)" should read -- (a) plus (c) --; Column 6, lines 12 - 25, in the Table, column 1, compound 7, "(a) plus (b)" should read -- (a) plus (d) --. Column 7, lines 36 - 45, in Table 1, column 1, compound 1, "0.00 g" should read -- 0.600 g --; Column 7, lines 36 - 45, in Table 1, column 2 under Fog, line 2, "0.2" should read -- 0.26 --; Column 7, lines 36 - 45, in Table 1, column 2 under Fog, line 4, "0.1" should read -- 0.16 --; Column 7, line 74, claim 1, "comprises" should read -- comprising --.

Column 10, lines

3 - 8, claim 8, the formula should appear as follows:



UNITED STATES PATENT OFFICE  
CERTIFICATE OF CORRECTION

Patent No. 3,732,104

Dated May 8, 1973

Inventor(s) HUBERT VANDENABEELE ET AL Page 2 of 2

It is certified that error appears in the above-identified patent and that said Letters Patent are hereby corrected as shown below:

Column 10, line 32, claim 11, after "stands for" insert -- lower alkyl carrying --; Column 10, lines 46 - 50, claim 12, the formula should appear as follows:



Column 8, line 35, "carying" should read -- carrying --; same line 35, after "carrying", second occurrence, insert -- the group  $R_3'CONH-$ , or a phenyl group, --.

Signed and sealed this 17th day of September 1974.

(SEAL)  
Attest:

McCOY M. GIBSON JR.  
Attesting Officer

C. MARSHALL DANN  
Commissioner of Patents